

June 25, 1929.

W. F. GRUPE

1,718,647

METHOD OF FORMING CORK FACINGS FOR LAUNDRY ROLLS

Filed Aug. 7, 1926



William F. Grupe,  
BY  
Henry J. Lueke,  
his ATTORNEY.

## UNITED STATES PATENT OFFICE.

WILLIAM F. GRUPE, OF LYNDHURST, NEW JERSEY, ASSIGNOR TO BOUCHER CORK COMPANY, OF NEW YORK, N. Y., A CORPORATION OF NEW YORK.

## METHOD OF FORMING CORK FACINGS FOR LAUNDRY ROLLS.

Application filed August 7, 1926. Serial No. 127,891.

This invention relates to an improved method of baking compressed products of cork.

My invention is directed particularly to the manufacture of baked compressed products such as cork envelopes for laundry rolls, flat-work ironers, mangles, and like machines wherein the baking of the compressed cork particles is carried out by applying the baking temperature directly at one side of the product and indirectly heating the other side or sides.

My method is applicable to cylindrical, i. e. annular envelopes for laundry rolls, as well to semi-cylindrical or other fractional portions of the full circumference, either formed originally in the baking operation or by severing the sections subsequent to the baking operation.

Further features and objects of the invention will be more fully understood from the following description and the accompanying drawings, in which

Fig. 1 is a central vertical sectional view of a mold and appurtenant devices for compressing the cork particles within the mold; this figure shows the mold at an intermediate stage of charging and compression;

Fig. 2 is a similar sectional view showing the mold completely charged with the compressed cork material;

Fig. 3 is a perspective view of a mold for the manufacture of full cylindrical envelopes for laundry rolls; and

Figs. 4 and 5 are respectively an end view and sectional side views of a battery of cylindrical molds enclosed in a single oven.

Referring to Figs. 1, 2 and 3, the mold and appurtenant parts are illustrated for use in the manufacture of annular envelopes of cork for laundry rolls and the like, and accordingly the mold proper 10 for deriving a full cylindrical cork roll as a completely molded product, comprises the outer cylindrical wall 11 and the inner cylindrical wall 12 and the bottom plate 13. Pursuant to my invention, the bottom plate 13 is annular, that is to say, is provided with a central opening 14 of a diameter as large as is practicable for attaining the desired strength of the material employed. If desired, the bottom wall portion 13 may be an extension of the outer wall 11

The open upper end of the mold 10 is utilized as the charging end, and is constructed to coact with a suitable charging chute, usually of cylindrical formation, and also combining with suitable compressing means and top closing means.

As one form of such arrangement, I have illustrated the charging chute 15 comprising the outer cylindrical wall 16 and inner cylindrical wall 17, the lower ends 16<sup>a</sup> and 17<sup>a</sup> being chamfered as indicated reversely to the chamfered of the outer and inner walls 11, 12, of the mold proper 10, to form a joint which is leak proof to the cork particles during the stages of charging and compression.

The charge of cork granules, flakes or the like is fed by means of a suitable delivery pipe into the charging chute 15 and the mold 10 is filled by successive stages of charging and compressing. For attaining such compression, I prefer the use of an annular ring 18, of steel or like metal, and a tampering element 19 in the form of a cylindrical shell of steel or the like, having inside and outside diameters conforming to the dimensions of the annular passage of the charging chute 15. The tampering element 19 is employed in conjunction with a hydraulic press or the like.

As indicated above, the mold proper 10 is charged by feeding the cork material into the chute 15 for a certain height of the material in the chute 15, whereupon the follower ring 18 and tampering element 19 are inserted in the annular passage of the chute 15 and the charge compressed for the desired degree of compression of the final cork product. Usually, the range of compression for laundry rolls is from a minimum value represented by the reduction in volume from two volumes to one volume to a maximum value represented by the reduction in volume from six to one. After such compressed partially filling charge of cork has been completed, fresh cork material is again fed into the chute 15, after withdrawal of the tampering element 19 and the follower plate 18, until the additional charge has been fed into the chute 15, whereupon the follower plate 18 and tampering element 19 are again placed into the chute 15, and the predetermined compression carried

out for the second charge installment. Such successive charging and compression stages are carried out until the mold is completely filled with the cork material at the predetermined compression. At such stage, the follower ring 18 assumes the position shown in Fig. 2, and the follower ring 18 now functions as the closure for the mold proper 10, and is retained in position by the use of the holding bars 20 of desired number and spaced about the circumference at the top of the mold 10. The bars 20 are inserted in the registering openings 21 of the outer wall 11 and the openings 22 of the inner wall 12. In Fig. 3 I have illustrated the mold proper 10 closed with its closure ring 18 by means of the holding bars 20, preparatory for the baking stage.

I prefer to bake the cork annulus from one side only, and usually from the inner side by reason of the more matured baking effect on the inner periphery of the resulting cork envelope and a less matured baking at the outer periphery of the cork envelope, whereby the resulting baked envelope possesses its highest degree of "sponginess" or resiliency under laundering conditions at its outer periphery, and a graduated degree of "sponginess" from the outer periphery toward the inner periphery.

Such product is further advantageous in that the portion of the annulus at the inner periphery is quite dense and highly resistant to moisture, attained by the increased hardness of the cork particles at the inner periphery effected by the application of the heat at the inner side. The application of the heat at the inner side of the cork envelope, during the baking stage, also effects the vaporization of the resin inherent in cork toward the outer periphery, thus increasing the resistance of the outer peripheral portion of the envelope against absorption of the moisture.

Usually, two or more envelopes, each of a complete circumference, are employed for each laundry roll. Preferably, the mold is rotated during the heating operation to equalize the baking action; the rotation of each mold and its compressed cork contents may be carried out in any suitable manner.

Any suitable method of applying the baking temperature may be employed. As an economical method of carrying out the baking operation, I have shown an oven, 23, which may be of rectangular shape, suitable for baking four envelope sections at a time.

As one advantageous form of carrying out the above noted operations and for attaining other results, I have indicated the skeletonized support 24 in which are journalled a pair of rollers 25 for rotatively supporting each mold 26, and each roll 25 extends lengthwise of the mold. As appears in Fig. 5, one roll of each set 25 may be positively driven, as by means of an electric motor 27, the shaft of which is connected directly or by gearing

28 to the respective sets of rolls 25, the other roll of each pair being idle, if desired. The heating unit 29 may be of the electrical type, as indicated, and each heating unit may be supported on a rod 30 of suitable insulating material, secured to and projecting from the rear wall 31 of the oven 23. The electrical insulating and wiring supporting base of each heating unit 29 may be of rectangular shape, as indicated. 75

The period of baking by heating from one side only of the mold is continued for a sufficient time to effect the desired rise of temperature at the outer peripheral portion of the cork charge within the respective molds. 80 Usually, the temperature of the outer portion of the mold charge is raised to a maximum of from 185° C. to 275° C.

My invention is applicable for other articles formed from baked, compressed cork particles, wherein the resiliency of the resulting article is desired to be of greater extent at one face, namely, the face disposed more remotely from the heating element in the baking operation. Such procedure also effects a resulting cork composition of greater baking effect at the face disposed adjacent to the heating element in the baking operation, such as the inner face of a cylindrical or other arcuate shape of cork envelope for a laundry roll, thereby insuring the absence of the penetration of any moisture or the like through the portion of the cork composition disposed more closely to the steel or other metallic laundry roll. 95

My method is also applicable for forming baked compressed cork articles of the flat padding type or partially arcuate padding type, as disclosed in my copending application Serial No. 51,753, filed by me on August 3rd, 1925 and Serial No. 5,089, filed by me on January 27th, 1925. In such embodiment of my invention, the cork envelope is compressed in a mold of corresponding shape, or the mold may be of flat formation, and the resulting flat cork products curved, or otherwise reshaped, as in a garment pressing machine, under the conditions of increased temperature and pressure by actual use in the machine. 105 110 115

Whereas, I have described my invention by reference to specific forms thereof, it will be understood that many changes and modifications may be made without departing from the spirit of the invention.

I claim:

1. The method of forming baked, compressed cork envelopes, which comprises compressing cork particles in an annular mold and baking the same by applying a higher temperature to one side of the mold than on the remaining sides of the mold, said higher temperature being capable of effecting the vaporization of the resin inherent in the cork particles. 125 130

2. The method of forming baked, compressed cork products, of arcuate shape, which comprises compressing cork particles in a mold of corresponding arcuate shape and baking the same by applying the heat directly to the side of less diameter of the resulting cork products.
3. The method of forming baked, com-
- pressed cork envelopes, which comprises compressing cork particles in an annular mold 10 and baking the same by applying the heat directly within the inner opening of the annular mold.

In testimony whereof I have signed this specification this 13th day of July, 1926.

WILLIAM F. GRUPE.